

# UNITED STATES PATENT OFFICE.

HARRY P. CORLISS, OF PITTSBURGH, PENNSYLVANIA, ASSIGNOR TO METALS RECOVERY COMPANY, OF NEW YORK, N. Y., A CORPORATION OF MAINE.

## FLOTATION OF MINERALS.

1,228,184.

Specification of Letters Patent. Patented May 29, 1917.

No Drawing.

Application filed March 21, 1917. Serial No. 156,492.

*To all whom it may concern:*

Be it known that I, HARRY P. CORLISS, a citizen of the United States, residing at Pittsburgh, in the county of Allegheny and State of Pennsylvania, have invented certain new and useful Improvements in Flotation of Minerals; and I do hereby declare the following to be a full, clear, and exact description of the invention, such as will enable others skilled in the art to which it appertains to make and use the same.

This invention relates to the concentration of minerals, such as sulfid ores and the like by flotation, and is based upon the discovery that improved results can be obtained by carrying out the flotation operation with the addition to the ore or mineral pulp of nitro-naphthalene, either alone or with added amounts of "oil." The nitro-naphthalene is a non-oleaginous solid material, which can nevertheless be distributed throughout the ore pulp with such uniformity that minimum amounts are required for effecting the concentration of the mineral by flotation. Nitro-naphthalene is obtainable, for example, from naphthalene by treatment with nitric acid.

In using the nitro-naphthalene it may be added to the ore, either alone or with added amounts of oil in any suitable manner so that it will be thoroughly and uniformly distributed throughout the ore pulp. The mixture is then subjected to a flotation operation as in an ordinary Calow cell or in an apparatus where the air is incorporated with the ore pulp by mechanical agitation. With some ore pulps it may be desirable to add either small amounts of acids or of alkalis depending upon the nature of the ore pulp to be treated.

The amount of nitro-naphthalene used may vary somewhat, for example between one-half pound and three or four pounds per ton of ore (that is, calculated on the weight of the ore and not of the ore pulp).

The results obtained by carrying on the flotation with the addition of nitro-naphthalene or with nitro-naphthalene and added oil indicate that higher grades of concentrates and better recoveries can be obtained than with the usual oil mixtures, and even with most, if not all, of the best oil mixtures.

It is a further characteristic of the invention that the froth obtained is readily broken up and the nitro-naphthalene recovered therefrom so that it is available for use in the treatment of further amounts of ore. That is to say the circuit water recovered from the concentrate and even that recovered from the tailings contains notable amounts of nitro-naphthalene which can thus be returned to the process with resulting economy in the amount required to be added for subsequent operations.

In applying the nitro-naphthalene it may be introduced into the tube mill in which the ore is being ground, or it may be otherwise introduced into the ore pulp in any suitable way, as, for instance, by first digesting it in hot water and mixing the product with the ore pulp just before it enters the flotation cell.

Having thus described my invention, what I claim is:

1. The method of effecting the concentration of minerals by flotation, which comprises adding to the mineral pulp a small amount of nitro-naphthalene and subjecting the resulting mixture to a flotation operation; substantially as described.

2. The method of effecting the concentration of minerals by flotation, which comprises adding to the mineral pulp a small amount of nitro-naphthalene and of oil and subjecting the resulting mixture to a flotation operation; substantially as described.

In testimony whereof I affix my signature.

HARRY P. CORLISS.